# EUROPEAN PATENT SPECIFICATION

(11) **EP 3 907 018 B1**
(45) Date of publication and mention of the grant of the patent: **29.03.2023**
(21) Application number: 21172009.9
(22) Date of filing: 04.05.2021
(51) Int. Cl.: B22C 7/02, B22C 9/04, B22C 9/08, B22C 9/10, B22C 21/14, B22D 15/00

(54) **THERMAL MANAGEMENT IN LOST WAX CASTING**
WÄRMEMANAGEMENT BEIM WACHSAUSSCHMELZGUSS
GESTION THERMIQUE DANS LA COULÉE À LA CIRE PERDUE

(30) Priority: 08.05.2020 US 202063022179 P
(43) Date of publication of application: 10.11.2021
(73) Proprietor: Hamilton Sundstrand Corporation, Charlotte, NC 28217-4578 (US)
(72) Inventor: MARCIN, John Joseph, Marlborough, 06447 (US)
(74) Representative: Dehns

(56) References cited:
- EP-A1- 2 792 771
- US-A1- 2017 087 626
- US-A1- 2019 358 850
- US-B2- 9 901 976

## Description

### BACKGROUND

The embodiments herein relate to casting of materials and more specifically to thermal management in lost wax casting.

Production of metal parts from lost-wax casting enables replication of parts on small and mass scales. Investment casting may include a wax part pattern of an article to be cast, which may be produced from a die mold. The component wax pattern may be connected with injected wax shapes on a wax assembly, which will typically possesses a pour-cup, down-sprue, wax in-gates, and then the component pattern itself. The wax tree, with the part patterns, is then coated with a ceramic slurry to form a ceramic shell over its surface.

After ceramic slurry application, the wax assembly may then be withdrawn from the slurry and dried. The steps of coating and drying are repeated until a ceramic shell mold around the wax tree is of a sufficient thickness, which may depend on the weight of the cast assembly. The wax tree, with the ceramic shell, is then placed in a furnace pressurized steam de-waxer vessel removes the wax from the inside of the ceramic mold. The ceramic mold is then placed into a furnace to heat and sinter the ceramic particles to strengthen the mold to enable the receipt of a certain volume of molten metal.

The hardening may be in a separate thermal processing step. The ceramic mold is then ready for the casting of the part. Molten metal is poured into the pour-cup and passed through the sprue and ingates into the component cavity once defined by the wax assembly. After the metal has solidified, the ceramic shell is removed mechanically to reveal the metal components on the assembly. The cast components are then removed from the assembly, mechanically finished and inspected. The ceramic shell is mechanically removed, e.g., by blunt force (or other mechanical action), after the metal is hardened.

For Solid mold casting, the wax tree is placed within a flask, which is then filled with the ceramic slurry. The flask, with the hardened ceramic, may be placed in a furnace and heated to remove the wax, and to harden the ceramic coating. The hardening may be in a separate heat-treating step. The ceramic mold is then ready for casting. In this form of casting, molten metal is also poured into the pour-cup and then passes into the down-sprue and runner system to feed the component pattern(s). The ceramic is also mechanically removed after the metal is solidified. Parts cast from these processes should be relatively defect free to meet manufacturing needs.

Patent documents US 2017/087626 A1, US 9 901 976 B2, US 2019/358850 A1 and EP 2 792 771 A1 relate to a lost-wax method of casting a product using inserts disposed inside the mould in order to control the thermal constraints during solidification.

### BRIEF SUMMARY

Disclosed is a lost-wax method of casting a product and a mould assembly as disclosed in appended claims 1-10.

### BRIEF DESCRIPTION OF THE DRAWINGS

The present disclosure is illustrated by way of example and not limited in the accompanying figures in which like reference numerals indicate similar elements.
FIG. 1 shows a wax assembly with temperature control elements according to an embodiment;
FIG. 2 shows the wax assembly encased in a ceramic mold as part of an investment casting process according to an embodiment;
FIG. 3 shows the wax assembly encased in the ceramic mold as part of a solid-mold casting process according to an embodiment;
FIG. 4 shows the ceramic mold, with the wax assembly removed, as part of an investment casting process according to an embodiment;
FIG. 5 shows the ceramic mold, with the wax assembly removed, as part of a solid-mold casting process according to an embodiment;
FIG. 6 shows the ceramic mold, including a sprue, a gate section and a part pattern chamber, filled with molten material as part of an investment casting process according to an embodiment;
FIG. 7 shows the ceramic mold, including a sprue, a gate section and a part pattern chamber, filled with molten material, as part of a solid-mold casting process according to an embodiment;
FIG. 8 shows a cast part, with the ceramic mold removed, as part of either the investment casting process or the solid mold process according to an embodiment;
FIG. 9 shows the cast part in a final form, with excess metal removed according to an embodiment; and
FIG. 10 is a flowchart showing a lost-wax method of casting a part according to an embodiment.

### DETAILED DESCRIPTION

A detailed description of one or more embodiments of the disclosed apparatus and method are presented herein by way of exemplification and not limitation with reference to the Figures.

During investment and solid mold type lost-wax casting, molten metal may undesirably solidify within the sprue, runners or assembly gating as well as within the component to which the assembly gating is attached before reaching the part pattern chamber. This may, result in casting defects which would cause the need for rework and repair, or would scrap the parts. In addition, the molten metal may cool unevenly within the part pattern chamber due to a variation of geometries within the part pattern chamber. For example, a relatively large mass of molten metal at thicker portions of a part pattern may result in an excess of heat in the same location compared with a thinner portion of the part pattern. Thus, thicker portions may cool more slowly than thinner portions of the part pattern within the part pattern chamber. The cooling dynamics may result in undesirable residual stress and strain in the final cast part.

As shown in FIG. 1, in view of the above identified concerns with lost wax investment and solid-mold type lost-wax casting, the disclosed embodiments utilize temperature control elements 100. The temperature control elements 100 take the form of thermal sink elements (or chillers) 100A1-100A5 (generally referenced as 100A). The thermal sink elements 100A are respectively applied to first portions 210A1, 210A2 (generally referenced as 210A) of a part pattern section 120 of a wax assembly 140 (or wax investment). As shown, the thermal sink elements 100A are applied to a side surface 125A, also referred to as an outer surface, of the part pattern section 120. However, the part pattern section 120 is three dimensional and thus has front and back surfaces 125B, 125C, identified schematically, and the thermal sink elements 100A may be applied there as well. For example, thermal sink elements 100A4, 100A5 are schematically shown for the front and back surfaces 125B, 125C, respectively.

The first portions 210A are relatively thick portions of the part pattern section 120 compared with, e.g., second portions 220B1, 220B2 (generally referenced as 220B) which may be near the respective first portions 210A. The thermal sink elements 100A are configured to provide for thermal control of the casting process by drawing out excess heat from molten material 180 utilized during the casting process. Faster solidification in areas of greater mass will result in more sound cast metal with less micro-porosity and macro-porosity defects. This is especially true if the area of larger mass is contained within regions of small mass where proper metal fill and solidification are not possible.

Additionally, the temperature control elements 100 take the form of insulating elements (or thermal barriers) 100B1-100B6 (generally referenced as 100B). The insulating elements 100B are respectively applied to a sprue pattern section 190 and gate-land pattern sections 200A1-200A4 (generally referenced as 200A) of a gate pattern section 130 of the wax assembly 140. Insulating sections may be required. The insulating elements 100B are configured to provide for thermal control of the casting process by preventing heat from being drawn out of the molten material 180 (FIGS. 6-7) applied during the casting process.

The thermal sink elements 100A are formed from conductive material such as metal or ceramic (SiC). The thermal sink elements 100A may have a higher thermal conductivity than the wax assembly 140 or a ceramic mold 150 (e.g., FIGS. 2-7) that is built around the wax assembly 140 as part of the casting process. The thermal sink elements 100A is attached directly to the part pattern section 120 of the wax assembly 140, to the ceramic mold 150, or to the gate pattern section 130 in close proximity to the part pattern section 120. The thermal sink elements 100A may extract heat relatively quickly from the part pattern chamber 160 (FIGS. 2-7) to provide a cast part 170 that is relatively sound and defect free.

The insulating elements 100B may be applied in similar fashion in the gate pattern section 130 to slow down the solidification process for fabricating the cast part 170. The insulating elements 100B is a ceramic with lower conductivity than the remainder of the ceramic mold 150. The insulating elements 100B may be formed of a material such as monolithic ceramics such as alumina, zircon, silica, etc., or a thermal barrier ceramic with controlled thermal conductivity such as yttria stabilized zirconia (YSZ), or a ceramic matrix composite which can control heat retention or dissipation in a controlled manner .

Thus, the disclosed process utilizes the temperature control elements 100 in situ in the investment casting and solid mold casting processes to affect a natural solidification rate of the molten material 180 (FIG. 8 and 9). The temperature control elements 100 may do this by directing and removing latent heat. This optimizes the solidification the molten material 180 to form a cast part 170 in the part pattern chamber 160. This process may improve product yields and reduce scrap and rework.

FIG. 2 shows an investment casting mold assembly 165 and includes the wax assembly 140 encased in the ceramic mold 150 as part of an investment casting process. FIG. 2 also shows the thermal sink elements 100A encased in the ceramic mold 150 and positioned against the part pattern section 120. The figure shows the insulating elements 100B encased in the ceramic mold 150 and located against the sprue pattern section 190.

FIG. 3 shows a solid-mold casting assembly 165A and includes the wax assembly 140 encased in the ceramic mold 150 as part of a solid-mold casting process. FIG. 3 also shows the thermal sink elements 100A encased in the ceramic mold 150 and located against the part pattern section 120. The figure also shows the insulating elements 100B encased in the ceramic mold 150 and located against the sprue pattern section 190 and the gate-land pattern sections 200A. FIG. 3 further shows the flask 230 for supporting the ceramic mold 150.

FIG. 4 shows the ceramic mold 150 with the wax assembly 140 removed as part of an investment casting process. FIG. 4 also shows the thermal sink elements 100A at the part pattern chamber 160, the insulating elements 100B at the sprue 190A and the gate-lands 200B1-200B5 (generally referenced as 200B) formed by removal of the wax assembly 140. FIG. 4 also shows the gate section 130A formed by removal of the wax assembly 140.

FIG. 5 shows the ceramic mold 150 with the wax assembly 140 removed as part of a solid-mold casting process. FIG. 5 also shows the thermal sink elements 100A at the part pattern chamber 160 formed by removal of the wax assembly 140, and the insulating elements 100B at the sprue 190A the gate-lands 200B formed by removal of the wax assembly 140. FIG. 5 further shows the gate section 130A formed by removal of the wax assembly 140 and the flask 230 for supporting the ceramic mold 150.

FIG. 6 shows the ceramic mold 150, including the sprue 190A, the gate section 130A and the part pattern chamber 160, filled with molten material 180 as part of an investment casting process. FIG. 6 also shows the thermal sink elements 100A at the part pattern chamber 160 and the insulating elements 100B at the sprue 190A and the gate-lands 200B.

FIG. 7 shows the ceramic mold 150, including the sprue 190A, the gate section 130A and the part pattern chamber 160, filled with molten material 180 as part of a solid-mold casting process. FIG. 7 also shows the thermal sink elements 100A at the part pattern chamber 160 and the insulating elements 100B at the sprue 190A and the gate-lands 200B. FIG. 7 further shows the flask 230 for supporting the ceramic mold 150.

The insulating elements 100B prevent the molten material 180 from cooling and drying, e.g., at the sprue 190A and the gate-lands 200B. The thermal sink elements 100A remove excess heat from molten material 180 in the part pattern chamber 160 adjacent to where it is placed. Thus, placing the thermal sink elements 100A next to a thicker portion of the part pattern chamber 160 enable cooling at a similar rate as a thinner portion of the part pattern chamber 160.

FIG. 8 shows the cast part 170 with the ceramic mold removed as part of either the investment casting process or the solid mold process. Excess metal 170A is around the cast part 170 in locations corresponding to the sprue 190A and gate section 130A (e.g., FIGS. 6-7). FIG. 9 shows the cast part 170 in the final form, with the excess metal 170A removed.

FIG. 10 is a flowchart showing a lost-wax method of casting a part, i.e., to provide the cast part 170. As shown in block 100, the method includes attaching the temperature control elements 100 to the wax assembly 140. As shown in block 110, the method includes encasing the wax assembly 140 and the temperature control elements 100 in the ceramic mold 150. As shown in block 120, the method includes removing the wax assembly 140 from the ceramic mold 150. As shown in block 130 in FIG. 10, the method includes filling the ceramic mold 150 with molten material 180 to form the cast part 170 within the ceramic mold 150. As shown in block 140 the method includes separating the ceramic mold 150 and the cast part 170 from each other.

Additionally, as shown in block 150, the method may further include attaching the thermal sink elements 100A to the part pattern section 120 of the wax assembly 140. As shown in block 160, the method may further include attaching the insulating elements 100B to the sprue pattern section 190 and the gate-land pattern sections 200A of the wax assembly 140.

As shown in block 170, the method further includes attaching steel blocks (as the thermal sink elements 100A) to the part pattern section of the wax assembly 140 to draw heat from the molten material 180. As shown in block 180, the method may include positioning the thermal sink elements 100A closer to the first portions 210A of the part pattern section 120 of the wax assembly 140 than the second portions 220A of the part pattern section 120 of the wax assembly 140. As indicated, the first portions 210A are thicker than the second portions 220A. As shown in block 200, the method may include positioning the thermal sink elements 100A about one or more of side, front and back surfaces 125A-125C of the wax assembly 140.

As shown in block 220, the method further includes attaching the temperature control elements 100 directly to the part pattern section 120 of the wax assembly 140. In such embodiment the thermal sink elements 100A may be formed of metal having a melting temperature that is greater than the molten material 180. Thus, when molten material 180 contacts the thermal sink elements 100A, the thermal sink elements 100A will remain solid and not contaminate the molten material 180. Similarly, the insulating elements 100B are also formed of a material that will not contaminate the molten material 180, and may be, e.g., a ceramic as indicated above. The temperature control elements 100 may be attached the wax assembly 140 via, e.g., additional melted wax.

In one embodiment, as shown in block 230, the method may include forming the ceramic mold 150 about the wax assembly 140 to a first thickness to define a first layer of the ceramic mold 150. The method may include, as shown in block 240, attaching the temperature control elements 100 to the first layer of the ceramic mold 150. In this embodiment, a thin layer of ceramic may separate the temperature control elements 100 from the wax assembly 140. This minimizes a likelihood of cross contamination between the molten material 180 and either of the temperature control elements 100.

As shown in block 250, the method may further include forming the ceramic mold 150 about the wax assembly 140 to a second thickness that is greater than the first thickness. This action encases the temperature control elements 100 within the ceramic mold 150. With this configuration, the temperature control elements 100 are securely contained and structurally isolated within the ceramic mold 150.

In one unclaimed embodiment, as shown in block 260, the method may further include forming layers of the ceramic mold 150 to build-up the ceramic mold 150 to the second thickness. This action forms the ceramic mold 150 about the wax assembly 140. Forming layers of the ceramic mold 150 may include encasing the wax assembly in a ceramic slurry, and drying the ceramic slurry, and repeating. In one embodiment, as shown in block 270, the method may further include positioning the wax assembly 140 in a flask 230. The method may further include, as shown in block 280, filling the flask 230 with the ceramic slurry. This action forms the ceramic mold 150 about the wax assembly 140.

As shown in block 290, the method may include mechanically separating, e.g., with application of blunt force (or other mechanical action, such as the utilization of a hammer or other impact implement), the ceramic mold 150 and the cast part 170 from each other. As shown in block 300, the method may further include thermally removing wax from and firing (e.g., applying fire or other similar heat source to) the ceramic mold 150 to sinter the ceramic and prepare the ceramic mold 150 for casting. Such heat treatment assists in strengthening the ceramic mold 150 so that it may withstand the temperature and the weight of the molten material 180.

The terminology used herein is for the purpose of describing particular embodiments only and is not intended to be limiting of the present disclosure. As used herein, the singular forms "a", "an" and "the" are intended to include the plural forms as well, unless the context clearly indicates otherwise. It will be further understood that the terms "comprises" and/or "comprising," when used in this specification, specify the presence of stated features, integers, steps, operations, elements, and/or components, but do not preclude the presence or addition of one or more other features, integers, steps, operations, element components, and/or groups thereof.

Those of skill in the art will appreciate that various example embodiments are shown and described herein, each having certain features in the particular embodiments, but the present disclosure is not thus limited. Rather, while various embodiments of the present disclosure have been described, it is to be understood that aspects of the present disclosure may include only some of the described embodiments. Accordingly, the present disclosure is not to be seen as limited by the foregoing description, but is only limited by the scope of the appended claims.

## Claims

1. A lost-wax method of casting a product, comprising:
attaching (100) temperature control elements (100) to a wax assembly (140), wherein the temperature control elements (100) include thermal sink elements (100A1-100A5) that are steel blocks of different sizes and insulating elements (100B) that are ceramic with a lower conductivity than the remainder of the ceramic mold, and
the method includes:
attaching the thermal sink elements (100A1-100A5) to a part pattern section (120) of the wax assembly (140), including side, front and back surfaces (125A, 125B, 125C) of the wax assembly (140);
positioning the thermal sink elements (100A1-100A5) closer to first portions (210A) of the part pattern section (120) of the wax assembly (140) than second portions (220A) of the part pattern section (120) of the wax assembly (140), wherein the first portions (210A) are thicker than the second portions (220A);
attaching the insulating elements (100B) to a sprue pattern section (190) and gate-land pattern sections (200A) of the wax assembly (140);
encasing (110) the wax assembly (140) and the temperature control elements (100) in a ceramic mold (150);
removing (120) the wax assembly (140) from the ceramic mold;
filling (130) the ceramic mold (150) with molten material to form a cast part within the ceramic mold (150); and
separating (140) the ceramic mold (150) and the cast part from each other.

2. The method of claim 1, wherein the method includes:
attaching the steel blocks to the part pattern section to draw heat from the molten material.

3. The method of any preceding claim, comprising:
attaching the temperature control elements directly to the wax assembly.

4. The method of any preceding claim, comprising:
forming the ceramic mold about the wax assembly to a first thickness to define a first layer of the ceramic mold; and
attaching the temperature control elements to the first layer of the ceramic mold.

5. The method of claim 4, comprising
forming the ceramic mold about the wax assembly to a second thickness that is greater than the first thickness to encase the temperature control elements within the ceramic mold.

6. The method of claim 5, further comprising
forming the ceramic mold about the wax assembly to the second thickness by repeatedly: drenching the wax assembly in a ceramic slurry; and drying the ceramic slurry.

7. The method of claim 5 or 6 further comprising
forming the ceramic mold about the wax assembly to the second thickness by:
positioning the wax assembly in a flask; and
filling the flask with a ceramic slurry.

8. The method of any preceding claim, further comprising
separating the ceramic mold and the cast part from each other by mechanical action, or including
thermally removing wax from and firing the ceramic mold to sinter the ceramic and prepare the ceramic mold for casting.

9. A mold assembly, comprising:
a wax assembly (140) including:
a part pattern section (120);
a gate pattern section (130) connected around an outer surface the part pattern section (120) and defining a sprue pattern section (190) and gate-land pattern sections (200A); and
temperature control elements (100) connected to the wax assembly (140),
wherein the temperature control elements (100) include thermal sink elements (100A1-100A5) that are steel blocks of different sizes and insulating
elements (100B) that are ceramic with a lower conductivity than the remainder of the ceramic mold,
the thermal sink elements (100A1-100A5) are attached to a part pattern section (120) of the wax assembly (140), including side, front and back surfaces (125A, 125B, 125C) of the wax assembly (140);
the thermal sink elements (100A1-100A5) are positioned closer to first portions (210A) of the part pattern section (120) of the wax assembly (140) than second portions (220A) of the part pattern section (120) of the wax assembly (140), wherein the first portions (210A) are thicker than the second portions (220A),
the insulating elements (100B) are attached to a sprue pattern section (190) and gate-land pattern sections (200A) of the wax assembly (140), and
wherein a ceramic mold (150) encases the wax assembly (140) and the temperature control elements (100).

10. The mold assembly of claim 9, wherein the temperature control elements are disposed between layers of ceramic in the ceramic mold.

## Patentansprüche

1. Wachsausschmelzverfahren zum Gießen eines Produkts, umfassend:
Anbringen (100) von Temperatursteuerelementen (100) an einer Wachsanordnung (140), wobei die Temperatursteuerelemente (100) Wärmesenkenelemente (100A1-100A5), die Stahlblöcke in unterschiedlichen Größen sind, und Isolierelemente (100B), die aus Keramik mit einer geringeren Leitfähigkeit als der Rest der Keramikform bestehen, beinhalten, und
wobei das Verfahren Folgendes beinhaltet:
Anbringen der Wärmesenkenelemente (100A1-100A5) an einem Teilmusterabschnitt (120) der Wachsanordnung (140), beinhaltend Seiten-, Vorder- und Rückflächen (125A, 125B, 125C) der Wachsanordnung (140);
Positionieren der Wärmesenkenelemente (100A1-100A5) näher an ersten Abschnitten (210A) des Teilmusterabschnitts (120) der Wachsanordnung (140) als an zweiten Abschnitten (220A) des Teilmusterabschnitts (120) der Wachsanordnung (140), wobei die ersten Abschnitte (210A) dicker als die zweiten Abschnitte (220A) sind;
Anbringen der Isolierelemente (100B) an einem Eingussmusterabschnitt (190) und Einguss-Steg-Musterabschnitten (200A) der Wachsanordnung (140);
Umschließen (110) der Wachsanordnung (140) und der Temperatursteuerelemente (100) in einer Keramikform (150);
Entfernen (120) der Wachsanordnung (140) aus der Keramikform;
Füllen (130) der Keramikform (150) mit geschmolzenem Material, um ein Gussteil innerhalb der Keramikform (150) zu bilden; und
Trennen (140) der Keramikform (150) und des Gussteils voneinander.

2. Verfahren nach Anspruch 1, wobei das Verfahren Folgendes beinhaltet:
Anbringen der Stahlblöcke an dem Teilmusterabschnitt, um dem geschmolzenen Material Wärme zu entziehen.

3. Verfahren nach einem der vorhergehenden Ansprüche, umfassend:
Anbringen der Temperatursteuerelemente direkt an der Wachsanordnung.

4. Verfahren nach einem der vorhergehenden Ansprüche, umfassend:
Bilden der Keramikform um die Wachsanordnung auf eine erste Dicke, um eine erste Schicht der Keramikform zu definieren; und
Anbringen der Temperatursteuerelemente an der ersten Schicht der Keramikform.

5. Verfahren nach Anspruch 4, umfassend
Bilden der Keramikform um die Wachsanordnung auf eine zweite Dicke, die größer als die erste Dicke ist, um die Temperatursteuerelemente innerhalb der Keramikform zu umschließen.

6. Verfahren nach Anspruch 5, ferner umfassend
Bilden der Keramikform um die Wachsanordnung auf die zweite Dicke durch wiederholtes: Tränken der Wachsanordnung in einer Keramikaufschlämmung; und Trocknen der Keramikaufschlämmung.

7. Verfahren nach Anspruch 5 oder 6, ferner umfassend Bilden der Keramikform um die Wachsanordnung auf die zweite Dicke durch:
Positionieren der Wachsanordnung in einem Kasten; und
Füllen des Kastens mit einer Keramikaufschlämmung.

8. Verfahren nach einem der vorhergehenden Ansprüche, ferner umfassend
Trennen der Keramikform und des Gussteils voneinander durch mechanische Einwirkung oder beinhaltend
thermischen Entfernens von Wachs von der Keramikform und Brennen dieser, um die Keramik zu sintern und die Keramikform zum Gießen vorzubereiten.

9. Formanordnung, umfassend:
eine Wachsanordnung (140), beinhaltend:
einen Teilmusterabschnitt (120);
einen Eingussmusterabschnitt (130), der um eine äußere Oberfläche des Teilmusterabschnitts (120) verbunden ist und einen Eingussmusterabschnitt (190) und Einguss-Steg-Musterabschnitte (200A) definiert; und
Temperatursteuerelemente (100), die mit der Wachsanordnung (140) verbunden sind,
wobei die Temperatursteuerelemente (100) Wärmesenkenelemente (100A1-100A5), die Stahlblöcke in unterschiedlichen Größen sind, und Isolierelemente (100B), die aus Keramik mit einer geringeren Leitfähigkeit als der Rest der Keramikform bestehen, beinhalten, die Wärmesenkenelemente (100A1-100A5) an einem Teilmusterabschnitt (120) der Wachsanordnung (140) angebracht sind, beinhaltend Seiten-, Vorder- und Rückflächen (125A, 125B, 125C) der Wachsanordnung (140);
wobei die Wärmesenkenelemente (100A1-100A5) näher an ersten Abschnitten (210A) des Teilmusterabschnitts (120) der Wachsanordnung (140) als an zweiten Abschnitten (220A) des Teilmusterabschnitts (120) der Wachsanordnung (140) positioniert sind, wobei die ersten Abschnitte (210A) dicker als die zweiten Abschnitte (220A) sind;
die Isolierelemente (100B) an einem Eingussmusterabschnitt (190) und Einguss-Steg-Musterabschnitten (200A) der Wachsanordnung (140) angebracht sind, und
wobei eine Keramikform (150) die Wachsanordnung (140) und die Temperatursteuerelemente (100) umschließt.

10. Formanordnung nach Anspruch 9, wobei die Temperatursteuerelemente zwischen Keramikschichten in der Keramikform angeordnet sind.

## Revendications

1. Procédé de cire perdue pour couler un produit, comprenant :
la fixation (100) d'éléments de régulation de température (100) à un ensemble de cire (140), dans lequel les éléments de régulation de température (100) comportent des éléments de dissipation thermique (100A1-100A5) qui sont des blocs d'acier de différentes tailles et des éléments isolants (100B) qui sont en céramique avec une conductivité plus faible que le reste du moule en céramique, et
le procédé comporte :
la fixation des éléments de dissipation thermique (100A1-100A5) à une section de modèle de pièce (120) de l'ensemble de cire (140), comportant des surfaces latérales, avant et arrière (125A, 125B, 125C) de l'ensemble de cire (140) ;
le positionnement des éléments de dissipation thermique (100A1-100A5) plus près des premières parties (210A) de la section de modèle de pièce (120) de l'ensemble de cire (140) que des secondes parties (220A) de la section de modèle de pièce (120) de l'ensemble de cire (140), dans lequel les premières parties (210A) sont plus épaisses que les secondes parties (220A) ;
la fixation des éléments isolants (100B) à une section de modèle de coulée (190) et à des sections de modèle grille-plateau (200A) de l'ensemble de cire (140) ;
l'enfermement (110) de l'ensemble de cire (140) et des éléments de régulation de température (100) dans un moule en céramique (150) ;
le retrait (120) de l'ensemble de cire (140) du moule en céramique ;
le remplissage (130) du moule en céramique (150) avec un matériau fondu pour former une pièce moulée à l'intérieur du moule en céramique (150) ; et
la séparation (140) du moule en céramique (150) et de la pièce coulée l'un de l'autre.

2. Procédé selon la revendication 1, dans lequel le procédé comporte :
la fixation des blocs d'acier à la section de modèle de pièce pour extraire la chaleur du matériau fondu.

3. Procédé selon une quelconque revendication précédente, comprenant :
la fixation des éléments de régulation de température directement à l'ensemble de cire.

4. Procédé selon une quelconque revendication précédente, comprenant :
la formation du moule en céramique autour de l'ensemble de cire à une première épaisseur pour définir une première couche du moule en céramique ; et
la fixation des éléments de régulation de température à la première couche du moule en céramique.

5. Procédé selon la revendication 4, comprenant la formation du moule en céramique autour de l'ensemble de cire à une seconde épaisseur qui est supérieure à la première épaisseur pour enfermer les éléments de régulation de température à l'intérieur du moule en céramique.

6. Procédé selon la revendication 5, comprenant en outre la formation du moule en céramique autour de l'ensemble de cire jusqu'à la seconde épaisseur en : trempant de manière répétée l'ensemble de cire dans une bouillie céramique ; et en séchant de manière répétée la bouillie céramique.

7. Procédé selon la revendication 5 ou 6 comprenant en outre la formation du moule en céramique autour de l'ensemble de cire à la seconde épaisseur en :
positionnant l'ensemble de cire dans un flacon ; et
remplissant le flacon avec une bouillie céramique.

8. Procédé selon une quelconque revendication précédente, comprenant en outre
la séparation du moule en céramique et de la pièce moulée l'un de l'autre par action mécanique, ou comportant
l'élimination thermique de la cire du moule en céramique et cuire le moule en céramique pour fritter la céramique et préparer le moule en céramique pour la coulée.

9. Ensemble de moule, comprenant :
un ensemble de cire (140) comportant :
une section de modèle de pièce (120) ;
une section de modèle de grille (130) connectée autour d'une surface extérieure à la section de modèle de pièce (120) et
définissant une section de modèle de coulée (190) et des sections de modèle de grille-plateau (200A) ; et
des éléments de régulation de température (100) connectés à l'ensemble de cire (140),
dans lequel les éléments de régulation de température (100) comportent des éléments de dissipation thermique (100A1-100A5) qui sont des blocs d'acier de différentes tailles et des éléments isolants (100B) qui sont en céramique avec une conductivité plus faible que le reste du moule en céramique,
les éléments de dissipation thermique (100A1-100A5) sont fixés à une section de modèle de pièce (120) de l'ensemble de cire (140), comportant des surfaces latérales, avant et arrière (125A, 125B, 125C) de l'ensemble de cire (140) ;
les éléments de dissipation thermique (100A1-100A5) sont positionnés plus près des premières parties (210A) de la section de modèle de pièce (120) de l'ensemble de cire (140) que des secondes parties (220A) de la section de modèle de pièce (120) de l'ensemble de cire (140), dans lequel les premières parties (210A) sont plus épaisses que les secondes parties (220A),
les éléments isolants (100B) sont fixés à une section de modèle de coulée (190) et à des sections de modèle grille-plateau (200A) de l'ensemble de cire (140), et
dans lequel un moule en céramique (150) renferme l'ensemble de cire (140) et les éléments de régulation de température (100).

10. Ensemble de moule selon la revendication 9, dans lequel les éléments de régulation de température sont disposés entre des couches de céramique dans le moule en céramique.
